



US008304152B2

(12) **United States Patent**  
**Wu**

(10) **Patent No.:** **US 8,304,152 B2**  
(45) **Date of Patent:** **Nov. 6, 2012**

(54) **SPIRODILACTAM POLYCARBONATE  
CONTAINING PHOTOCOCONDUCTORS**

(75) Inventor: **Jin Wu**, Pittsford, NY (US)

(73) Assignee: **Xerox Corporation**, Norwalk, CT (US)

(\*) Notice: Subject to any disclaimer, the term of this patent is extended or adjusted under 35 U.S.C. 154(b) by 245 days.

(21) Appl. No.: **12/846,023**

(22) Filed: **Jul. 29, 2010**

(65) **Prior Publication Data**

US 2012/0028180 A1 Feb. 2, 2012

(51) **Int. Cl.**

**G03G 5/047** (2006.01)  
**G03G 5/05** (2006.01)

(52) U.S. Cl. .... **430/58.8**; 430/59.6; 430/96; 430/58.75

(58) **Field of Classification Search** .... 430/59.6,  
430/96, 58.8, 58.75

See application file for complete search history.

(56) **References Cited**

U.S. PATENT DOCUMENTS

4,906,725 A 3/1990 Wang  
5,030,707 A 7/1991 Wang  
5,095,088 A 3/1992 Want

5,128,436 A \* 7/1992 Wang ..... 528/96  
5,521,306 A 5/1996 Burt et al.  
6,080,833 A \* 6/2000 Otsuji et al. ..... 528/201  
6,913,863 B2 7/2005 Wu et al.  
2005/0106483 A1 \* 5/2005 Shoshi et al. ..... 430/58.7  
2006/0105254 A1 5/2006 Wu et al.

OTHER PUBLICATIONS

Zhou, Hui et al. "New spirodilactam polymers" Polymer (vol. 47), pp. 6927-6930 (2006).\*

Jin Wu et al., U.S. Appl. No. 12/644,071 on Polyalkylene Glycol Benzoate Containing Photoconductors, filed Dec. 22, 2009.

Jin Wu, U.S. Appl. No. 12/768,873 on Dendritic Polyester Polyol Photoconductors, filed Apr. 28, 2010.

Jin Wu et al., U.S. Appl. No. 12/550,498 on Plasticizer Containing Photoconductors, filed Aug. 31, 2009.

Robert C.U. Yu et al., U.S. Appl. No. 12/471,311 on Flexible Imaging Members Having a Plasticized Imaging Layer, filed May 22, 2009.

Robert C.U. Yu et al., U.S. Appl. No. 12/434,572 on Flexible Imaging Members Without Anticurl Layer, filed May 1, 2009.

\* cited by examiner

*Primary Examiner* — Christopher Rodee

(74) *Attorney, Agent, or Firm* — Eugene O. Palazzo

(57) **ABSTRACT**

A photoconductor that includes a supporting substrate, an optional ground plane layer, an optional hole blocking layer, an optional adhesive layer, a photogenerating layer, and at least one charge transport layer, and where the charge transport layer contains a spirodilactam based polycarbonate.

**32 Claims, No Drawings**

## 1

SPIRODILACTAM POLYCARBONATE  
CONTAINING PHOTOCONDUCTORSCROSS REFERENCE TO RELATED  
APPLICATIONS

Copending U.S. application Ser. No. 12/644,071, filed Dec. 22, 2009, the disclosure of which is totally incorporated herein by reference, illustrates a photoconductor that includes a supporting substrate, an optional ground plane layer, an optional hole blocking layer, a photogenerating layer, and at least one charge transport layer, and where the charge transport layer contains a polyalkylene glycol benzoate.

Illustrated in copending U.S. application Ser. No. 12/768,873, filed Apr. 28, 2010, the disclosure of which is totally incorporated herein by reference, is a photoconductor comprising a substrate, and an undercoat layer thereover comprised of a metal oxide and a mixture of a phenolic resin and a dendritic polyester polyol; a photogenerating layer; and a charge transport layer.

U.S. application Ser. No. 12/550,498, filed Aug. 31, 2009, the disclosure of which is totally incorporated herein by reference, illustrates a photoconductor comprising a substrate, a photogenerating layer, and a charge transport layer, and wherein the charge transport layer contains a cyclohexanedicarboxylate, such as diisononyl cyclohexanedicarboxylate.

U.S. application Ser. No. 12/471,311, filed May 22, 2009, the disclosure of which is totally incorporated herein by reference, illustrates a flexible imaging member comprising a flexible substrate; a charge generating layer disposed on the substrate; and at least one charge transport layer disposed on the charge generating layer, wherein the charge transport layer comprises a polycarbonate, N,N'-diphenyl-N,N'-di(3-methylphenyl)-1,1-biphenyl-4,4'-diamine, a first plasticizer or a second plasticizer, and further wherein the first plasticizer and the second plasticizer are miscible with both the polycarbonate and N,N'-diphenyl-N,N'-di(3-methylphenyl)-1,1-biphenyl-4,4'-diamine.

U.S. application Ser. No. 12/434,572, filed May 1, 2009, illustrates an imaging member comprising a substrate; a charge generating layer disposed on the substrate; and at least one charge transport layer disposed on the charge generating layer, wherein the charge transport layer comprises a polycarbonate, a charge transport compound of N,N'-diphenyl-N,N'-bis(3-methylphenyl)-1,1-biphenyl-4,4'-diamine, and a liquid compound having a high boiling point, and further wherein the liquid compound is miscible with both the polycarbonate and N,N'-diphenyl-N,N'-bis(3-methylphenyl)-1,1-biphenyl-4,4'-diamine.

Examples of plasticizers illustrated in the appropriate above copending applications are, for example, dioctyl phthalate, diallyl phthalate, liquid styrene dimer, and others as illustrated by the structure/formulas disclosed.

High photosensitivity titanyl phthalocyanines are illustrated in copending U.S. application Ser. No. 10/992,500, U.S. Publication No. 20060105254, which, for example, discloses a process for the preparation of a Type V titanyl phthalocyanine, comprising providing a Type I titanyl phthalocyanine; dissolving the Type I titanyl phthalocyanine in a solution comprising a trihaloacetic acid and an alkylene halide like methylene chloride; adding the resulting mixture comprising the dissolved Type I titanyl phthalocyanine to a solution comprising an alcohol and an alkylene halide thereby precipitating a Type Y titanyl phthalocyanine; and treating the Type Y titanyl phthalocyanine with monochlorobenzene to yield a Type V titanyl phthalocyanine.

## 2

A number of the components of the above cross referenced applications, the disclosures of each being totally incorporated herein by reference in their entireties, such as the appropriate supporting substrates, resin binders, antioxidants, charge transport components, titanyl phthalocyanines, high photosensitivity titanyl phthalocyanines, such as Type V, hydroxygallium phthalocyanines, chlorogallium phthalocyanines, adhesive layers, and the like, may be selected for the photoconductors and imaging members of the present disclosure in embodiments thereof.

## BACKGROUND

This disclosure is generally directed to layered imaging members, photoreceptors, photoconductors, and the like that can be selected for a number of systems, such as copiers and printers, especially xerographic copiers and printers inclusive of digital printers, and printers that generate color xerographic documents, and which printers can be selected for the office environment, and for production and commercial uses. More specifically, the present disclosure is directed to multi-layered drum, or flexible belt imaging members or devices comprised of a supporting medium like a substrate; an optional ground plane layer, an optional hole blocking layer; a photogenerating layer; and a charge transport layer, including at least one or a plurality of charge transport layers, and wherein at least one charge transport layer is, for example, from 1 to about 7, from 1 to about 3, and one; and more specifically, a first charge transport layer and a second charge transport layer, and where a spirodilactam based polycarbonate, and yet more specifically, a first charge transport resin binder of a copolymer of a spirodilactam polycarbonate and a polycarbonate together with a second polycarbonate. The spirodilactam based polycarbonates containing photoconductors possess, in embodiments, excellent wear characteristics, and where the spirodilactam based polycarbonates function, for example, as a charge transport layer (CTL) first or second resin binder, and an additional binder of, for example, a polycarbonate.

Yet more specifically, an advantage of the photoconductors, in embodiments of the present disclosure, is that the wear rates when selecting for the charge transport layer a spirodilactam based polycarbonate was, for example, about 38 nanometers/kilocycle, about 40 percent less than that of a charge transport layer (CTL) with no spirodilactam based polycarbonates, where the wear rate is about 58 nanometers/kilocycle.

The photoconductors disclosed herein possess a number of advantages especially in xerographic processes and xerographic printers, such as, in embodiments, the minimal wearing of the charge transport layer or layers; the minimization or substantial elimination of undesirable ghosting on developed images, such as xerographic images, including decreased ghosting at various relative humidities; excellent cyclic and stable electrical properties; minimal charge deficient spots (CDS); compatibility with the photogenerating and charge transport resin binders; extended xerographic biased charge roller (BCR) wear characteristics and acceptable lateral charge migration (LCM) characteristics, such as for example, excellent LCM resistance.

Ghosting refers, for example, to when a photoconductor is selectively exposed to positive charges in a number of xerographic print engines, and where some of the positive charges enter the photoconductor and manifest themselves as a latent image in the subsequent printing cycles. This print defect can cause a change in the lightness of the half tones, and is commonly referred to as a "ghost" that is generated in the

previous printing cycle. An example of a source of the positive charges is the stream of positive ions emitted from the transfer corotron. Since the paper sheets are situated between the transfer corotron and the photoconductor, the photoconductor is shielded from the positive ions from the paper sheets. In the areas between the paper sheets, the photoconductor is fully exposed, thus in this paper free zone the positive charges may enter the photoconductor. As a result, these charges cause a print defect or ghost in a half tone print if one switches to a larger paper format that covers the previous paper print free zone.

Excellent cyclic stability of the photoconductor refers, for example, to almost no or minimal change in a generated known photoinduced discharge curve (PIDC), especially no or minimal residual potential cycle up after a number of charge/discharge cycles of the photoconductor, for example about 100 kilocycles, or xerographic prints of, for example, from about 80 to about 100 kiloprints. Excellent color print stability refers, for example, to substantially no or minimal change in solid area density, especially in 60 percent halftone prints, and no or minimal random color variability from print to print after a number of xerographic prints, for example 50 kiloprints.

Also included within the scope of the present disclosure are methods of imaging and printing with the photoconductor devices illustrated herein. These methods generally involve the formation of an electrostatic latent image on the imaging member, followed by developing the image with a toner composition comprised, for example, of thermoplastic resin, colorant, such as pigment, charge additive, and surface additive, reference U.S. Pat. Nos. 4,560,635; 4,298,697 and 4,338,390, the disclosures of which are totally incorporated herein by reference, subsequently transferring the toner image to a suitable image receiving substrate, and permanently affixing the image thereto. In those environments wherein the photoconductor is to be used in a printing mode, the imaging method involves the same operation with the exception that exposure can be accomplished with a laser device or image bar. More specifically, the flexible photoconductor belts disclosed herein can be selected for the Xerox Corporation iGEN® machines that generate with some versions over 100 copies per minute. Processes of imaging, especially xerographic imaging and printing, including digital and/or color printing, are thus encompassed by the present disclosure. The imaging members are, in embodiments, sensitive in the wavelength region of, for example, from about 400 to about 900 nanometers, and in particular from about 650 to about 850 nanometers, thus diode lasers can be selected as the light source. Moreover, the imaging members of this disclosure are useful in color xerographic applications, particularly high-speed color copying and printing processes inclusive of digital xerographic processes.

## REFERENCES

There is illustrated in U.S. Pat. No. 6,913,863 a photoconductive imaging member comprised of a hole blocking layer, 5 a photogenerating layer, and a charge transport layer, and wherein the hole blocking layer is comprised of a metal oxide; and a mixture of a phenolic compound and a phenolic resin wherein the phenolic compound contains at least two phenolic groups.

10 A number of layered photoconductors are known and have been described in numerous U.S. patents, and which patents disclose, for example, a photoconductor comprised of a supporting substrate, a photogenerating layer, and a charge transport layer and where the photogenerating layer and charge transport layer include certain resin binders, such as polycarbonates, polyesters, and the like.

15 Illustrated in U.S. Pat. No. 5,521,306 is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine which can be selected as a photoconductor photogenerating pigment. Processes for the generation of hydroxy gallium phthalocyanines are also illustrated in U.S. Pat. Nos. 5,482,811 and 5,473,064.

20 The appropriate components, such as the supporting substrates, the photogenerating layer components, the charge transport layer components, the overcoating layer components, and the like of the above-recited patents may be selected for the photoconductors of the present disclosure in embodiments thereof.

25

## EMBODIMENTS

30 In aspects thereof of the present disclosure, there is illustrated a photoconductor comprising a supporting substrate, a photogenerating layer, and a charge transport layer, and 40 wherein the charge transport layer contains a spirodilactam polycarbonate copolymer binder; a photoconductor comprised in sequence of a supporting substrate, a hole blocking layer thereover, an adhesive layer, a photogenerating layer, and a charge transport layer, and wherein the charge transport layer contains a charge transport component, a spirodilactam polycarbonate present in an amount of from about 1 to about 45 20 weight percent, and a polycarbonate present in an amount of from about 40 to about 65 weight percent; a photoconductor comprised of a photogenerating layer comprised of a photogenerating pigment, a hole blocking layer, an adhesive layer, and a charge transport layer, and wherein the charge transport layer is comprised of a charge transport component, 50 a spirodilactam polycarbonate copolymer represented by



5



-continued

6



20

wherein x and y represent mole percent, and where the sum of x and y thereof is 100 mole percent, and a polycarbonate selected from the group consisting of poly(4,4'-dihydroxy-diphenyl-1-1-cyclohexane), poly(4,4'-isopropylidene-diphenyl) carbonate, and mixtures thereof; a photoconductor comprising a substrate, a photogenerating layer, and a charge transport layer, and wherein the charge transport layer contains a charge transport component, such as an aryl amine and other known charge and hole transport components, a resin binder, and a spirodilactam polycarbonate, such as those disclosed in U.S. Pat. Nos. 4,906,725; 5,030,707 and 5,095,088, the disclosures of which are totally incorporated herein by reference in their entireties; a photoconductor comprising a substrate, an undercoat layer thereover, a photogenerating layer, and at least one charge transport layer, and wherein the at least one charge transport layer in contact with the photogenerating layer contains a spirodilactam based polycarbonate present in an amount of from about 1 to about 80 weight percent, from 2 to about 50 weight percent, from about 3 to about 20 weight percent, and more specifically about 6 weight percent, a second resin binder, like a polycarbonate dissimilar than the spirodilactam polycarbonate present in an amount of from about 1 to about 80 weight percent, from about 20 to about 70 weight percent, from about 40 to about 60 weight percent, and more specifically about 54 weight percent; a photoconductor comprised in sequence of a photogenerating layer comprised of a photogenerating pigment, and a hole transport layer, and wherein the transport layer is comprised of a hole transport component, a polycarbonate and a copolymer of a spirodilactam polycarbonate and a polycarbonate; a photoconductor comprising a supporting substrate, a ground plane layer, a hole blocking layer, an adhesive layer, a photogenerating layer comprised of at least one photogenerating pigment, and a charge transport layer comprised of at least one charge transport component, and where the charge transport layer has incorporated therein a hole transport component, a polycarbonate, and a copolymer of a spirodilactam polycarbonate and a known polycarbonate, that is the same as the polycarbonate included in known charge transport layers; a flexible photoconductive member comprised in sequence of a supporting substrate, a ground plane layer, a hole blocking or undercoat layer, a photogenerating layer thereover comprised of at least one photogenerating pigment, and as a second binder for the charge transport layer a spirodilactam based polycarbonate; a photoconductor which includes a hole blocking layer and an adhesive layer where the adhesive layer

is situated between the hole blocking layer and the photogenerating layer, and the hole blocking layer is situated between the supporting substrate layer, and the adhesive layer; a photoconductor comprising a supporting substrate, a hole blocking layer, a photogenerating layer, and at least one charge transport layer comprised of at least one charge transport component, and wherein a first pass charge transport layer is in contact with the photogenerating layer, and a second pass charge transport layer is in contact with the first charge transport layer, and the second top charge transport layer includes therein a spirodilactam based polycarbonate, a hole transport component, and a resin binder; a photoconductor comprising a supporting substrate, a photogenerating layer in contact with the supporting substrate, and at least one charge transport layer in contact with the photogenerating layer, and wherein at least one, such as 1, 2, or 3 charge transport layers, contains a polymer of a spirodilactam polycarbonate, and a polycarbonate as illustrated herein; a photoconductor comprised in sequence of a photogenerating layer comprised of a photogenerating pigment, such as a hydroxygallium phthalocyanine, a chlorogallium phthalocyanine or a titanyl phthalocyanine, a first charge transport layer, and a second charge transport layer thereover, and wherein the second charge transport layer is comprised of a charge transport component, a resin binder, a first resin binder of a copolymer of a spirodilactam polycarbonate and a polycarbonate, and as a second resin binder a copolymer of a spirodilactam polycarbonate and a polycarbonate; or where the second charge transport layer is comprised of a charge transport component, a resin binder, a first resin binder of a copolymer of a spirodilactam polycarbonate and a polycarbonate, and a second resin binder of polycarbonate Z, where the copolymer of a spirodilactam polycarbonate and a polycarbonate minimizes the wear of the charge transport layer; a photoconductor wherein the spirodilactam is 1,6-di(4-hydroxyphenyl)-1,6-diazoaspiro[4.4]nonane-2,7-dione, 1,6-di(4-hydroxyphenyl)-3,4,8,9-tetrafluoro-1,6-diazoaspiro[4.4]nonane-2,7-dione, 1,6-di(3-hydroxy-4-chlorophenyl)-3,3,4,4,8,8,9, or 9-octylmethyl-1,6 diazoaspiro[4.4]nonane-2,7-dione; and the polycarbonate binder is a poly(4,4'-dihydroxy-diphenyl-1-1-cyclohexane), a poly(4,4'-isopropylidene-diphenylene) carbonate, a poly(4,4'-cyclohexylidene diphenylene) carbonate, or a poly(4,4'-isopropylidene-3,3'-dimethyl-diphenyl) carbonate; and a photoconductor comprised of a photogenerating layer comprised of a photogenerating pigment, a hole blocking layer, an adhesive layer, and a charge transport layer,

and wherein the charge transport layer is comprised of a charge transport component, a spirodilactam polycarbonate copolymer represented by



wherein x and y represent mole percents, and where the sum of x and y thereof is 100 mole percent, and a polycarbonate selected from the group consisting of poly(4,4'-dihydroxy-diphenyl-1,1-cyclohexane), poly(4,4'-isopropylidene-diphenyl) carbonate, and mixtures thereof.

The photoconductors disclosed herein in embodiments include in the charge transport layer a copolymer of a spirodilactam polycarbonate and a polycarbonate as illustrated in U.S. Pat. Nos. 4,906,725; 5,030,707 and 5,095,088, the disclosures of which are totally incorporated herein by reference in their entireties, and more specifically, the copolymers of a spirodilactam polycarbonate and a polycarbonate, and yet more specifically, where the copolymer of a spirodilactam polycarbonate and a polycarbonate is represented, for example, by

wherein x and y represent the mole percent, and more specifically, where x is from about 1 to about 30 mole percent (from about to about includes between about and about), from

about 2 to about 20 mole percent, from about 1 to about 5 mole percent, from about 3 to about 10 mole percent, or other suitable mole percents, and y is, for example, from about 70 to 99 mole percent, from about 80 to about 98 mole percent, from about 99 to about 95 mole percent, from about 90 to about 97 mole percent, or other suitable mole percents, and with, for example, a weight average molecular weight of from about 10,000 to about 100,000, from about 20,000 to about 75,000, from about 35,000 to about 90,000 as determined by known analytic processes, such as by GPC, and where the copolymers of the referenced spirodilactam polycarbonate and polycarbonate are available from Shell Development Company, Houston, Tex.



In embodiments, specific examples of copolymers of spirodilactam polycarbonate and a polycarbonate can be represented by



wherein x and y represent the mole percents of each segment in brackets, and more specifically, where x is, for example, from about 1 to about 30 mole percent (from about to about includes all values or numbers in between about and about), from about 2 to about 20 mole percent, or from about 3 to about 10 mole percent, and y is, for example, from about 70 to 99 mole percent, from about 80 to about 98 mole percent, or from about 90 to about 97 mole percent, and with, for example, a weight average molecular weight as illustrated here, such as for example, from about 10,000 to about 100,000.

Examples of spirodilactams are 1,6-di(4-hydroxyphenyl)-1,6-diazoaspiro[4.4]nonane-2,7-dione, 1,6-di(4-hydroxyphenyl)-3,4,8,9-tetrafluoro-1,6-diazoaspiro[4.4]nonane-2,7-dione, 1,6-di(3-hydroxy-4-chlorophenyl)-3,3,4,4,8,8,9, or 9-octylmethyl-1,6-diazoaspiro[4.4]nonane-2,7-dione; and examples of spirodilactam polycarbonate copolymers are a polycarbonate copolymer of a spirodilactam, and a bisphenol selected, for example, from the group consisting of bisphenol A and bisphenol Z, and said polycarbonate binder is a poly(4,4'-dihydroxy-diphenyl-1-1-cyclohexane, a poly(4,4'-isopropylidene-diphenylene) carbonate, a poly(4,4'-cyclohexylidene-diphenylene) carbonate, a poly(4,4'-isopropylidene-3,3'-dimethyl-diphenyl) carbonate, or mixtures thereof.

The polycarbonate second resin binder and the polycarbonate selected for forming the spirodilactam polymer possesses, for example, a number average molecular weight ( $M_n$ ) of, for example, from about 10,000 to about 80,000, or from about 20,000 to about 60,000, and a weight average molecular weight ( $M_w$ ) of from about 20,000 to about 100,000, or from about 40,000 to about 80,000, where  $M_w$  and  $M_n$  were determined by Gel Permeation Chromatography (GPC). Specific examples of the second polycarbonate resin, a number of which are prepared, for example, from di(hydroxyphenyl) alkanes, such as 2,2-di(4-hydroxyphenyl)propane, are illustrated in U.S. Pat. No. 5,030,707, the disclosure of which is totally incorporated herein by reference, like PCZ-400 [poly(4,4'-dihydroxy-diphenyl-1-1-cyclohexane,  $M_n=40,000$ )] available from Mitsubishi Gas Chemical Company, Ltd.; poly(4,4'-isopropylidene-diphenylene) carbonate (also referred to

as bisphenol-A-polycarbonate), poly(4,4'-cyclohexylidene diphenylene) carbonate (also referred to as bisphenol-Z-polycarbonate), poly(4,4'-isopropylidene-3,3'-dimethyl-diphe-

nyl) carbonate (also referred to as bisphenol-C-polycarbonate), and the like, and mixtures thereof, and other known suitable polycarbonates.

#### Photoconductor Layer Examples

A number of known components can be selected for the various photoconductor layers, such as the supporting substrate, the photogenerating layer, the charge transport layer, the hole blocking layer when present, and the adhesive layer when present, such as those components as illustrated in the copending applications referenced herein.

The thickness of the photoconductor substrate layer depends on many factors, including economical considerations, electrical characteristics, adequate flexibility, availability, and cost of the specific components for each layer, and the like, thus this layer may be of a substantial thickness, for example about 3,000 microns, such as from about 1,000 to about 2,000 microns, from about 500 to about 1,000 microns, or from about 300 to about 700 microns ("about" throughout includes all values in between the values recited), or of a minimum thickness. In embodiments, the thickness of this layer is from about 75 to about 300 microns, or from about 100 to about 150 microns.

The photoconductor substrate may be opaque or substantially transparent, and may comprise any suitable material including known or future developed materials. Accordingly, the substrate may comprise a layer of an electrically nonconductive or conductive material such as an inorganic or an organic composition. As electrically nonconducting materials, there may be employed various resins known for this purpose including polyesters, polycarbonates, polyamides, polyurethanes, and the like, which are flexible as thin webs. An electrically conducting substrate may be any suitable metal of, for example, aluminum, nickel, steel, copper, gold, and the like, or a polymeric material, as described above, filled with an electrically conducting substance, such as carbon, metallic powder, and the like, or an organic electrically conducting material. The electrically insulating or conductive substrate may be in the form of an endless flexible belt, a web,

## 11

a rigid cylinder, a sheet, and the like. The thickness of the substrate layer depends on numerous factors, including strength desired, and economical considerations. For a drum, this layer may be of a substantial thickness of, for example, up to many centimeters or of a minimum thickness of less than a millimeter. Similarly, a flexible belt may be of a substantial thickness of, for example, about 250 microns, or of a minimum thickness of less than about 50 microns provided there are no adverse effects on the final electrophotographic device.

In embodiments, where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, supporting substrate layers selected for the photoconductors of the present disclosure, and which substrates can be opaque or substantially transparent comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

Examples of electrically conductive layers or ground plane layers usually present on nonconductive substrates are gold, gold containing compounds, aluminum, titanium, titanium/zirconium, and other known suitable known components. The thickness of the metallic ground plane is, for example, from about 10 to about 100 nanometers, from about 20 to about 50 nanometers, and more specifically, about 35 nanometers, and the titanium or titanium/zirconium ground plane is, for example, from about 10 to about 30 nanometers, and more specifically, about 20 nanometers in thickness.

An optional hole blocking layer when present is usually in contact with the ground plane, and can be comprised of a number of known components as illustrated herein, such as metal oxides, phenolic resins, aminosilanes, mixtures thereof, and the like.

Aminosilane examples included in the hole blocking layer can be represented by



wherein  $\text{R}_1$  is an alkylene group containing, for example, from 1 to about 25 carbon atoms;  $\text{R}_2$  and  $\text{R}_3$  are independently selected from the group consisting of at least one of hydrogen or alkyl containing, for example, from 1 to about 12 carbon atoms, and more specifically, from 1 to about 4 carbon atoms; aryl with, for example, from about 6 to about 42 carbon atoms, such as a phenyl group; and a poly(alkylene like eth-

## 12

ylene amino) group; and  $\text{R}_4$ ,  $\text{R}_5$  and  $\text{R}_6$  are independently selected from an alkyl group containing, for example, from 1 to about 10 carbon atoms, and more specifically, from 1 to about 4 carbon atoms.

- 5 Aminosilane specific examples include 3-aminopropyl triethoxysilane, N,N-dimethyl-3-aminopropyl triethoxysilane, N-phenylaminopropyl trimethoxysilane, triethoxysilylpropylethylene diamine, trimethoxysilylpropylethylene diamine, trimethoxysilylpropylethylene triamine, N-aminoethyl-3-aminopropyl trimethoxysilane, N-2-aminoethyl-3-aminopropyl trimethoxysilane, N-2-aminoethyl-3-aminopropyl tris(ethylethoxy)silane, p-aminophenyl trimethoxysilane, N,N'-dimethyl-3-aminopropyl triethoxysilane, 3-aminopropylmethyl diethoxysilane, 3-aminopropyl trimethoxysilane, N-methylaminopropyl triethoxysilane, methyl[2-(3-trimethoxysilylpropylamino)ethylamino]-3-propionate, (N,N'-dimethyl-3-amino)propyl triethoxysilane, N,N-dimethylaminophenyl triethoxysilane, trimethoxysilylpropylethylene triamine, and the like, and mixtures thereof.
- 10 Yet more specific aminosilane materials are 3-aminopropyl triethoxysilane (y-APS), N-aminoethyl-3-aminopropyl trimethoxysilane, (N,N'-dimethyl-3-amino)propyl triethoxysilane, and mixtures thereof.

25 The aminosilane may be hydrolyzed to form a hydrolyzed silane solution before being added into the final undercoat coating solution or dispersion. During hydrolysis of the aminosilanes, the hydrolyzable groups, such as alkoxy groups, are replaced with hydroxyl groups. The pH of the hydrolyzed silane solution can be controlled to obtain excellent characteristics on curing, and to result in electrical stability. A solution pH of, for example, from about 4 to about 10 can be selected, and more specifically, a pH of from about 7 to about 8. Control of the pH of the hydrolyzed silane solution may be affected with any suitable material, such as generally organic or inorganic acids. Typical organic and inorganic acids include acetic acid, citric acid, formic acid, hydrogen iodide, phosphoric acid, hydrofluorosilicic acid, p-toluene sulfonic acid, and the like.

30 The hole blocking layer can, in embodiments, be prepared by a number of known methods, the process parameters being dependent, for example, on the photoconductor member desired. The hole blocking layer can be coated as a solution or a dispersion onto the supporting substrate or on to the ground plane layer by the use of a spray coater, dip coater, extrusion coater, roller coater, wire-bar coater, slot coater, doctor blade coater, gravure coater, and the like, and dried at from about 40° C. to about 200° C. for a suitable period of time, such as from about 1 minute to about 10 hours, under stationary conditions or in an air flow. The coating can be accomplished to provide a final coating thickness of, for example, from about 0.01 to about 30 microns, or from about 0.02 to about 5 microns, or from about 0.03 to about 0.5 micron after drying.

35 Generally, the photogenerating layer can contain known photogenerating pigments, such as metal phthalocyanines, metal free phthalocyanines, alkylhydroxyl gallium phthalocyanines, hydroxygallium phthalocyanines, chlorogallium phthalocyanines, perylenes, especially bis(benzimidazo) perylene, titanyl phthalocyanines, and the like, and more specifically, vanadyl phthalocyanines, Type V hydroxygallium phthalocyanines, high sensitivity titanyl phthalocyanines, and inorganic components such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers, and the amount

of photogenerating material contained in the photogenerating layer. Accordingly, this layer can be of a thickness of, for example, from about 0.05 to about 10 microns, and more specifically, from about 0.25 to about 2 microns when, for example, the photogenerating compositions are present in an amount of from about 30 to about 75 percent by volume. The maximum thickness of this layer, in embodiments, is dependent primarily upon factors, such as photosensitivity, electrical properties, and mechanical considerations.

The photogenerating composition or pigment can be present in a resinous binder composition in various amounts inclusive of up to 100 percent by weight. Generally, however, from about 5 to about 95 percent by volume of the photogenerating pigment is dispersed in about 95 to about 5 percent by volume of the resinous binder, or from about 20 to about 30 percent by volume of the photogenerating pigment is dispersed in about 70 to about 80 percent by volume of the resinous binder composition. In one embodiment, about 90 percent by volume of the photogenerating pigment is dispersed in about 10 percent by volume of the resinous binder composition, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of coating solvents for the photogenerating layer are ketones, alcohols, aromatic hydrocarbons, halogenated aliphatic hydrocarbons, ethers, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like, hydrogenated amorphous silicon and compounds of silicon and germanium, carbon, oxygen, nitrogen, and the like fabricated by vacuum evaporation or deposition. The photogenerating layer may also comprise inorganic pigments of crystalline selenium and its alloys; Groups II to VI compounds; and organic pigments such as quinacridones, polycyclic pigments such as dibromoanthrone pigments, perylene and perinone diamines, polynuclear aromatic quinones, azo pigments including bis-, tri- and tetrakis-azos, and the like dispersed in a film forming polymeric binder, and fabricated by solvent coating techniques.

In embodiments, examples of polymeric binder materials that can be selected as the matrix or binder for the photogenerating layer are thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene, acrylonitrile copolymers, poly(vinyl chloride), vinyl chloride and vinyl acetate copolymers, acrylate copolymers, alkyd resins, cellulosic film formers, poly(amideimide), styrene butadiene copolymers, vinylidene chloride-vinyl chloride

copolymers, vinyl acetate-vinylidene chloride copolymers, styrene-alkyd resins, poly(vinyl carbazole), and the like. These polymers may be block, random, or alternating copolymers.

Various suitable and conventional known processes may be used to mix, and thereafter apply the photogenerating layer coating mixture like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like.

The final dry thickness of the photogenerating layer is as illustrated herein, and can be, for example, from about 0.01 to about 30 microns after being dried at, for example, about 40° C. to about 150° C. for about 15 to about 90 minutes. More specifically, a photogenerating layer of a thickness, for example, of from about 0.1 to about 10 microns, or from about 0.2 to about 2 microns can be applied to or deposited on a supporting substrate, or on other surfaces in between the substrate and the charge transport layer, and the like. A charge blocking layer or hole blocking layer may optionally be applied to the electrically conductive supporting substrate surface prior to the application of a photogenerating layer. When desired, an adhesive layer may be included between the charge blocking, hole blocking layer or interfacial layer, and the photogenerating layer. Usually, the photogenerating layer is applied onto the supporting substrate or the blocking layer when it is present, and a charge transport layer or plurality of charge transport layers is formed on the photogenerating layer. This structure may have the photogenerating layer on top of or below the charge transport layer.

In embodiments, a suitable known adhesive layer can be included in the photoconductor. Typical adhesive layer materials include, for example, polyesters, polyurethanes, and the like. The adhesive layer thickness can vary, and in embodiments is, for example, from about 0.05 to about 0.3 micron. The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like.

As an optional adhesive layer or layers usually in contact with or situated between the hole blocking layer and the photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

A number of charge transport compounds can be included in the charge transport layer, which layer generally is of a thickness of from about 5 to about 75 microns, and more specifically, of a thickness of from about 10 to about 40 microns. Examples of charge transport components are aryl amines of the following formulas/structures



wherein X is a suitable hydrocarbon like alkyl, alkoxy, aryl, and derivatives thereof; a halogen, or mixtures thereof, and especially those substituents selected from the group consisting of Cl and CH<sub>3</sub>; and molecules of the following formulas



wherein X, Y and Z are independently alkyl, alkoxy, aryl, a halogen, or mixtures thereof, and wherein at least one of Y and Z are present.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxy, and aryls can also be selected in embodiments.

Examples of specific aryl amines that can be selected for the charge transport layer include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, N,N'-bis(4-butylphenyl)-N,N'-bis(3-chlorophenyl)-[p-terphenyl]-4,4'-diamine; hydrazones such as N-phenyl-N-methyl-3-(9-ethyl) carbazyl hydrazone and 4-diethyl amino benzaldehyde-1,2-diphenyl hydrazone; and oxadiazoles such as 2,5-bis(4-N,N'-diethylaminophenyl)-1,2,4-oxadiazole, stilbenes, and the like. However, in embodiments, to minimize or avoid cycle-up in equipment, such as printers with high throughput, the charge transport layer should be substantially free (less than about two percent) of di or triamino-triphenyl methane. A small molecule charge transporting compound that permits injection of holes into the photogenerating layer with high

Other known charge transport layer molecules can be selected reference for example, U.S. Pat. Nos. 4,921,773 and 4,464,450, the disclosures of which are totally incorporated herein by reference.

- 5 In addition to the compatible spirodilactam based polycarbonates, examples of additional binder materials selected for the charge transport layer or layers include polycarbonates, polyarylates, acrylate polymers, vinyl polymers, cellulose polymers, polyesters, polysiloxanes, polyamides, polyurethanes, poly(cyclo olefins), epoxies, and random or alternating copolymers thereof; and more specifically, polycarbonates such as poly(4,4'-isopropylidene-diphenylene) carbonate (also referred to as bisphenol-A-polycarbonate), poly(4,4'-cyclohexylidene diphenylene) carbonate (also referred to as bisphenol-Z-polycarbonate), poly(4,4'-isopropylidene-3,3'-dimethyl-diphenyl) carbonate (also referred to as bisphenol-C-polycarbonate), and the like. In embodiments, electrically inactive binders are comprised of polycarbonate resins with a weight average molecular weight M<sub>w</sub> of 10 from about 20,000 to about 100,000, or with a molecular weight M<sub>w</sub> of from about 50,000 to about 100,000. Generally, the transport layer contains from about 10 to about 75 percent by weight of the charge transport material, and more specifically, from about 35 to about 50 percent of this material.
- 15 20 25 The charge transport layer or layers, and more specifically, a first charge transport in contact with the photogenerating layer, and thereover a top or second charge transport overcoating layer, may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9

efficiency, and transports them across the charge transport layer with short transit times includes N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, and N,N'-diphenyl-N,N'-bis(3-chlorophenyl)-[p-terphenyl]-4,4'-diamine, or mixtures thereof. If desired, the charge transport material in the charge transport layer may comprise a polymeric charge transport material, or a combination of a small molecule charge transport material and a polymeric charge transport material.

Examples of components or materials optionally incorporated into the charge transport layers, or at least one charge transport layer to, for example, enable excellent lateral charge migration (LCM) resistance include hindered phenolic antioxidants, such as tetrakis methylene(3,5-di-tert-butyl-4-hydroxy hydrocinnamate) methane (IRGANOX<sup>TM</sup> 1010, available from Ciba Specialty Chemical), butylated hydroxytoluene (BHT), and other hindered phenolic antioxidants including SUMILIZER<sup>TM</sup> BHT-R, MDP-S, BBM-S, WX-R, NR, BP-76, BP-101, GA-80, GM and GS (available from Sumitomo Chemical Co., Ltd.), IRGANOX<sup>TM</sup> 1035, 1076, 1098, 1135, 1141, 1222, 1330, 1425WL, 1520L, 245, 259, 3114, 3790, 5057 and 565 (available from Ciba Specialties Chemicals), and ADEKA STAB<sup>TM</sup> AO-20, AO-30, AO-40, AO-50, AO-60, AO-70, AO-80 and AO-330 (available from Asahi Denka Co., Ltd.); hindered amine antioxidants such as SANOL<sup>TM</sup> LS-2626, LS-765, LS-770 and LS-744 (available from SNKYO CO., Ltd.), TINUVIN<sup>TM</sup> 144 and 622LD (available from Ciba Specialties Chemicals), MARK<sup>TM</sup> LA57, LA67, LA62, LA68 and LA63 (available from Asahi Denka Co., Ltd.), and SUMILIZER<sup>TM</sup> TPS (available from Sumitomo Chemical Co., Ltd.); thioether antioxidants such as SUMILIZER<sup>TM</sup> TP-D (available from Sumitomo Chemical Co., Ltd.); phosphite antioxidants such as MARK<sup>TM</sup> 2112, PEP-8, PEP-24G, PEP-36, 329K and HP-10 (available from Asahi Denka Co., Ltd.); other molecules such as bis(4-diethylamino-2-methylphenyl)phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layers is from about 0 to about 20 weight percent, from about 1 to about 10 weight percent, or from about 3 to about 8 weight percent.

A number of processes may be used to mix, and thereafter apply the charge transport layer or layers coating mixture to the photogenerating layer. Typical application techniques include spraying, dip coating, roll coating, wire wound rod coating, and the like. Drying of the charge transport deposited coating may be effected by any suitable conventional technique such as oven drying, infrared radiation drying, air drying, and the like.

The thickness of each of the charge transport layers, in embodiments, is from about 10 to about 70 microns, but thicknesses outside this range may, in embodiments, also be selected. The charge transport layer should be an insulator to

the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to 200:1, and in some instances 400:1. The charge transport layer is substantially nonabsorbing to visible light or radiation in the region of intended use, but is electrically "active" in that it allows the injection of photogenerated holes from the photoconductive layer, or photogenerating layer, and allows these holes to be transported to selectively discharge a surface charge present on the surface of the photoconductor. Typical application techniques include spraying, dip coating, roll coating, wire wound rod coating, and the like. Drying of the deposited coating may be effected by any suitable conventional technique, such as oven drying, infrared radiation drying, air drying, and the like. A known optional overcoating may be applied over the charge transport layer to provide abrasion protection.

In embodiments, the present disclosure relates to a photoconductive imaging member comprised of a titanium/zirconium containing ground plane layer, a hole blocking layer, a photogenerating layer, a polycarbonate charge transport layer, and an overcoating spirodilactam based polycarbonate containing charge transport layer as illustrated herein a photoconductive member with a photogenerating layer of a thickness of from about 0.1 to about 8 microns, and at least one transport layer each of a thickness of from about 5 to about 100 microns; an imaging method and an imaging apparatus containing a charging component, a development component, a transfer component, and a fixing component, and wherein the apparatus contains a photoconductive imaging member comprised of a supporting substrate, a ground plane layer, a hole blocking layer, and thereover a photogenerating layer comprised of a photogenerating pigment, and a charge transport layer or layers, and thereover an overcoating charge transport layer, and where the transport layer is of a thickness of from about 40 to about 75 microns; a member wherein the photogenerating layer contains a photogenerating pigment present in an amount of from about 8 to about 95 weight percent; a member wherein the thickness of the photogenerating layer is from about 0.1 to about 4 microns; a member wherein the photogenerating layer contains a polymer binder; a member wherein the binder is present in an amount of from about 50 to about 90 percent by weight, and wherein the total of all layer components is about 100 percent; a member wherein the photogenerating component is a titanyl phthalocyanine or a hydroxygallium phthalocyanine that absorbs light of a wavelength of from about 370 to about 950 nanometers; an imaging member wherein the supporting substrate is comprised of a conductive substrate comprised of a metal; an imaging member wherein the conductive substrate is aluminum, aluminized polyethylene terephthalate, aluminized polyethylene naphthalate, titanized polyethylene terephthalate, titanized polyethylene naphthalate, titanized/zirconized polyethylene terephthalate, titanized/zirconized polyethylene naphthalate, goldized polyethylene terephthalate, or goldized polyethylene naphthalate; an imaging member wherein the photogenerating resinous binder is selected from the group consisting of polyesters, polyvinyl butyral, polycarbonates, polystyrene-b-polyvinyl pyridine, and polyvinyl

formals; an imaging member wherein the photogenerating pigment is a metal free phthalocyanine; an imaging member wherein a single charge transport layer or where each of the charge transport layers comprises



wherein X is selected from the group consisting of alkyl, alkoxy, aryl, and halogen; an imaging member wherein alkyl and alkoxy contains from about 1 to about 12 carbon atoms; an imaging member wherein alkyl contains from about 1 to about 5 carbon atoms; an imaging member wherein alkyl is methyl; an imaging member wherein each of, or at least one of the charge transport layers comprises



wherein X and Y are independently alkyl, alkoxy, aryl, a halogen, or mixtures thereof; an imaging member wherein alkyl and alkoxy for the charge transport component aryl amine contain from about 1 to about 12 carbon atoms; an imaging member wherein alkyl contains from about 1 to about 5 carbon atoms, and wherein the resinous binder is selected from the group consisting of polycarbonates and polystyrene; an imaging member wherein the photogenerating pigment present in the photogenerating layer is comprised of chlorogallium phthalocyanine, or Type V hydroxygallium phthalocyanine prepared by hydrolyzing a gallium phthalocyanine precursor by dissolving the hydroxygallium phthalocyanine in a strong acid, and then reprecipitating the resulting dissolved precursor in a basic aqueous media; removing any ionic species formed by washing with water; concentrating the resulting aqueous slurry comprised of water and hydroxygallium phthalocyanine to a wet cake; removing water from the wet cake by drying; and subjecting the resulting dry pigment to mixing with the addition of a second

solvent to cause the formation of the hydroxygallium phthalocyanine; an imaging member wherein the Type V hydroxygallium phthalocyanine has major peaks, as measured with an X-ray diffractometer, at Bragg angles (2 theta)+/-0.2°) 5 7.4, 9.8, 12.4, 16.2, 17.6, 18.4, 21.9, 23.9, 25.0, 28.1 degrees, and the highest peak at 7.4 degrees; a method of imaging which comprises generating an electrostatic latent image on an imaging member developing the latent image, and transferring the developed electrostatic image to a suitable substrate; a method of imaging wherein the imaging member is exposed to light of a wavelength of from about 370 to about 950 nanometers; a photoconductive member wherein the photogenerating layer is situated between the substrate and the charge transport; a member wherein the charge transport 10 layer is situated between the substrate and the photogenerating layer; a member wherein the photogenerating layer is of a thickness of from about 0.1 to about 50 microns; a member wherein the photogenerating pigment is dispersed in from about 1 weight percent to about 80 weight percent of a polymer binder; a member wherein the photogenerating binder is present in an amount of from about 50 to about 90 percent by weight, and wherein the total of the layer components is about 15 100 percent; an imaging member wherein the photogenerating component is Type V hydroxygallium phthalocyanine, 20 Type V titanyl phthalocyanine or chlorogallium phthalocyanine, and the charge transport layer contains a hole transport of N,N'-diphenyl-N,N'-bis(3-methylphenyl)-1,1'-biphenyl-4, 25 4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine. N,N'-bis(4-butylphenyl)-N,N'-bis(4-isopropylphenyl)-[p-terphenyl]-4, 30 4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, N,N'-diphenyl-N,N'-bis(3-chlorophenyl)-[p-terphenyl]-4,4'-diamine molecules, and wherein the hole 35 transport resinous binder is selected from the group consisting of polycarbonates and polystyrene; an imaging member 40 wherein the photogenerating layer contains a metal free phthalocyanine; a photoconductor wherein the photogenerating layer contains an alkoxygallium phthalocyanine; photoconductive imaging members comprised of a supporting substrate, a photogenerating layer, a hole transport layer, and in 45 embodiments wherein a plurality of charge transport layers are selected, such as for example, from two to about ten, and more specifically two, may be selected; and a photoconductive imaging member comprised of an optional supporting substrate, a photogenerating layer, and a first, second, and 50 third charge transport layer.

In embodiments, the charge transport component can be represented by the following formulas/structures



**21****22**

-continued



The following Examples are being submitted to illustrate embodiments of the present disclosure. Molecular weights were determined by Gel Permeation analysis.

#### COMPARATIVE EXAMPLE 1

On a 30 millimeter thick aluminum drum substrate, an undercoat layer was prepared and deposited thereon as follows.

Zirconium acetylacetone tributoxide (35.5 parts),  $\gamma$ -aminopropyl triethoxysilane (4.8 parts), and poly(vinyl butyral)

BM-S (2.5 parts) were dissolved in n-butanol (52.2 parts). The resulting solution was then coated by a dip coater on the above aluminum drum substrate, and the coating solution

<sup>60</sup> layer was preheated at 59° C. for 13 minutes, humidified at 58° C. (dew point=54° C.) for 17 minutes, and dried at 135° C. for 8 minutes. The thickness of the resulting undercoat layer was approximately 1.3 microns.

A photogenerating layer, 0.2 micron in thickness, comprising chlorogallium phthalocyanine (Type C) was deposited on the above undercoat layer. The photogenerating layer coating

23

dispersion was prepared as follows. 2.7 Grams of chlorogallium phthalocyanine (ClGaPc) Type C pigment were mixed with 2.3 grams of the polymeric binder (carboxyl-modified vinyl copolymer, VMCH, available from Dow Chemical Company), 15 grams of n-butyl acetate, and 30 grams of xylene. The resulting mixture was mixed in an Attritor mill with about 200 grams of 1 millimeter Hi-Bea borosilicate glass beads for about 3 hours. The dispersion mixture obtained was then filtered through a 20 micron Nylon cloth filter, and the solids content of the dispersion was diluted to about 6 weight percent.

Subsequently, a 32 micron charge transport layer was coated on top of the above photogenerating layer from a solution prepared by dissolving N,N'-diphenyl-N,N-bis(3-methylphenyl)-1,1'-biphenyl-4,4'-diamine (mTBD, 4 grams), and a film forming polymer binder PCZ-400 [poly(4,

24

transport layer PCZ-400/spirodilactam polycarbonate copolymer/4,4'-diamine ratio was 54/6/40.

## EXAMPLE II

A photoconductor is prepared by repeating the process of Comparative Example 1 except that a 32 micron thick charge transport layer is coated on top of the photogenerating layer from a solution prepared from N,N'-diphenyl-N,N-bis(3-methylphenyl)-1,1'-biphenyl-4,4'-diamine (4 grams), the film forming polymer binder PCZ-400[poly(4,4'-dihydroxy-diphenyl-1-1-cyclohexane carbonate,  $M_w = 40,000$ )], available from Mitsubishi Gas Chemical Company, Ltd. (5.4 grams), and a copolymer of a spirodilactam polycarbonate, and a polycarbonate, which copolymer is represented by, as obtained from Shell Development Company, Houston Tex.,



4'-dihydroxy-diphenyl-1-1-cyclohexane,  $M_w = 40,000$ ], available from Mitsubishi Gas Chemical Company, Ltd. (6 grams) in a solvent mixture of 21 grams of tetrahydrofuran (THF), and 9 grams of toluene, followed by drying in an oven at about 120° C. for about 40 minutes. The resulting charge transport layer PCZ-400/mTBD ratio was 60/40.

## EXAMPLE I

A photoconductor was prepared by repeating the process of Comparative Example 1 except that a 32 micron thick charge transport layer was coated on top of the photogenerating layer from a solution prepared from N,N'-diphenyl-N,N-bis(3-methylphenyl)-1,1'-biphenyl-4,4'-diamine (4 grams), the film forming polymer binder PCZ-400 [poly(4,4'-dihydroxy-diphenyl-1-1-cyclohexane carbonate,  $M_w = 40,000$ )], available from Mitsubishi Gas Chemical Company, Ltd. (5.4 grams), a copolymer of a spirodilactam polycarbonate, and a polycarbonate, which copolymer was represented by

30 wherein x is equal to 10 mole percent, y is equal to 90 mole percent, and with a weight average molecular weight of 100,000 (0.6 gram) dissolved in a solvent mixture of 21 grams of tetrahydrofuran (THF) and 9 grams of toluene. The charge 35 transport layer PCZ-400/spirodilactam polycarbonate copolymer/4,4'-diamine ratio is 54/6/40.

## EXAMPLE III

A photoconductor is prepared by repeating the process of Comparative Example 1 except that a 32 micron thick charge transport layer is coated on top of the photogenerating layer from a solution prepared from N,N'-diphenyl-N,N-bis(3-methylphenyl)-1,1'-biphenyl-4,4'-diamine (4 grams), the film forming polymer binder PCZ-400 [poly(4,4'-dihydroxy-



wherein x is equal to 6 mole percent, y is equal to 94 mole percent, and with a weight average molecular weight of 60,000 (0.6 gram), dissolved in a solvent mixture of 21 grams of tetrahydrofuran (THF), and 9 grams of toluene. The charge

65 diphenyl-1-1-cyclohexane carbonate,  $M_w = 40,000$ ], available from Mitsubishi Gas Chemical Company, Ltd. (5.4 grams), a copolymer of a spirodilactam polycarbonate, and a polycarbonate, which copolymer is represented by



wherein x is equal to 20 mole percent, y is equal to 80 mole percent, and with a weight average molecular weight of 80,000 (0.6 gram) dissolved in a solvent mixture of 21 grams of tetrahydrofuran (THF), and 9 grams of toluene. The charge transport layer PCZ-400/spirodilactam polycarbonate copolymer/4,4'-diamine ratio is 54/6/40.

#### Electrical Property Testing

The above prepared photoconductors of Comparative Example 1 and Example I were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic curves from which the photosensitivity and surface potentials at various exposure intensities were measured. Additional electrical characteristics were obtained by a series of charge-erase cycles with incrementing surface potential to generate several voltage versus charge density curves. The scanner was equipped with a scorotron set to a constant voltage charging at various surface potentials. The above photoconductors were tested at surface potentials of 700 volts with the exposure light intensity incrementally increased by means of regulating a series of neutral density filters; and the exposure light source was a 780 nanometer light emitting diode. The xerographic simulation was completed in an environmentally controlled light tight chamber at ambient conditions (40 percent relative humidity and 22° C.).

Substantially similar PIDCs were obtained for the above two photoconductors. Therefore, the incorporation of the above copolymer of a spirodilactam polycarbonate and a polycarbonate into the charge transport layer did not adversely affect the electrical properties of the Example I photoconductor.

#### Wear Testing

Wear tests of the photoconductors of Comparative Example 1 and Example I were performed using an in-house wear test fixture (biased charging roll, BCR charging, and peak to peak voltage of 1.45 kilovolts). The total thickness of each photoconductor was measured by a Permascope before

each wear test was initiated. Then the photoconductors were separately placed into the wear fixture for 50 kilocycles. The total photoconductor thickness was measured again with the Permascope, and the difference in thickness was used to calculate wear rate (nanometers/kilocycle) of the photoconductors. The smaller the wear rate, the more wear resistant was the photoconductor. The wear rate data is summarized in Table 1.

25

TABLE 1

|                       | Wear Rate<br>(Nanometers/Kilocycle) |
|-----------------------|-------------------------------------|
| Comparative Example 1 | 58                                  |
| Example I             | 38                                  |

35

The photoconductor of Example I exhibited an about 40 percent lower wear rate than the photoconductor of Comparative Example 1 (38 nanometers/kilocycle for the Example I photoconductor versus 58 nanometers/kilocycle for the Comparative Example 1 photoconductor). Incorporation of the spirodilactam polycarbonate copolymer into the charge transport layer thus reduced the wear rate.

45

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, position, size, shape, angle, color, or material.

50

55

What is claimed is:

1. A photoconductor comprising a supporting substrate, a photogenerating layer, and a charge transport layer, and wherein said charge transport layer contains a spirodilactam polycarbonate copolymer binder.
2. A photoconductor in accordance with claim 1 wherein said copolymer is represented by the following

60

65



and wherein x and y represent mole percents, and where the sum thereof is about 100 mole percent, and where said charge transport layer further includes a second binder of a polycarbonate.

3. A photoconductor in accordance with claim 2 wherein x is from about 1 to about 30 mole percent, y is from about 70 to about 99 mole percent; and said charge transport layer is comprised of a hole transport component, said spirodilactam polycarbonate copolymer, and said polycarbonate.

4. A photoconductor in accordance with claim 2 wherein said second polycarbonate binder is poly(4,4'-dihydroxy-diphenyl-1-1-cyclohexane) carbonate, poly(4,4'-isopropylidene-diphenylene) carbonate, poly(4,4'-cyclohexylidene diphenylene) carbonate, or poly (4,4'-isopropylidene-3,3'-dimethyl-diphenyl) carbonate.

8. A photoconductor in accordance with claim 2 wherein said spirodilactam copolymer is present in an amount of from about 2 to about 10 weight percent, and said second polycarbonate binder is present in an amount of from about 40 to about 60 weight percent.

9. A photoconductor in accordance with claim 2 wherein said charge transport layer is comprised of a first charge transport layer in contact with said photogenerating layer, and a second charge transport layer in contact with said first charge transport layer, and wherein said spirodilactam copolymer, and said second polycarbonate binder are present in said second charge transport layer.

10. A photoconductor in accordance with claim 2 wherein said spirodilactam copolymer is represented by one of the following



5. A photoconductor in accordance with claim 2 wherein for said spirodilactam copolymer x is from about 2 to about 20 mole percent, and y is from about 80 to about 98 mole percent, and wherein the total thereof is 100.

6. A photoconductor in accordance with claim 2 wherein said spirodilactam copolymer possesses a weight average molecular weight of from about 25,000 to about 200,000, and a number average molecular weight of from about 20,000 to about 150,000.

7. A photoconductor in accordance with claim 2 wherein said spirodilactam copolymer is present in an amount of from about 1 to about 20 weight percent of the charge transport layer components.

55 wherein x and y represent mole percents, and where the sum thereof is 100 mole percent; wherein said x is a number between about 2 and about 10, and said y is a number from between about 90 and about 98, and said charge transport layer is comprised of said copolymer, aryl amines, and said second polycarbonate of poly(4,4'-dihydroxy-diphenyl-1-1-cyclohexane) carbonate, poly(4,4'-isopropylidene-diphenylene) carbonate, poly(4,4'-cyclohexylidene diphenylene) carbonate or poly(4,4'-isopropylidene-3,3'-dimethyl-diphenyl) carbonate.

60 11. A photoconductor in accordance with claim 2 wherein said spirodilactam copolymer present in an amount of from about 2 to about 20 weight percent is represented by the following formulas/structures

29



30



or



wherein x and y represent the mole percents, and where the sum thereof is 100 mole percent, and said second polycarbonate binder is poly(4,4'-dihydroxy-diphenyl-1-1-cyclohexane carbonate, poly(4,4'-isopropylidene-diphenylene) carbonate, poly(4,4'-cyclohexylidene diphenylene) carbonate, or poly(4,4'-isopropylidene-3,3'-dimethyl-diphenyl) carbonate each present in an amount of from about 45 to about 65 weight percent.

12. A photoconductor in accordance with claim 2 wherein said second polycarbonate binder is poly(4,4'-dihydroxy-diphenyl-1-1-cyclohexane) carbonate, poly(4,4'-isopropylidene-diphenylene) carbonate, poly(4,4'-cyclohexylidene diphenylene) carbonate, or poly(4,4'-isopropylidene-3,3'-dimethyl-diphenyl) carbonate; said charge transport layer includes

-continued



or



31

wherein X, Y, and Z are independently selected from the group consisting of alkyl, alkoxy, aryl, halogen, and mixtures thereof, and x and y of said copolymer are from about 40 to about 60 mole percent.

13. A photoconductor in accordance with claim 2 wherein said charge transport layer includes a component selected from the group consisting of N,N'-bis(methylphenyl)-1,1-biphenyl-4,4'-diamine, tetra-p-tolyl-biphenyl-4,4'-diamine, N,N'-diphenyl-N,N'-bis(4-methoxyphenyl)-1,1-biphenyl-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-



4,4'-diamine, and N,N'-diphenyl-N,N'-bis(3-chlorophenyl)-[p-terphenyl]-4,4'-diamine, and wherein x and y of said copolymer are from about 40 to about 60 mole percent.

14. A photoconductor in accordance with claim 2 wherein said photogenerating layer is comprised of at least one photogenerating pigment.

15. A photoconductor in accordance with claim 14 wherein said photogenerating pigment is comprised of at least one of a titanyl phthalocyanine, a hydroxygallium phthalocyanine, a halogallium phthalocyanine, a bisperylene, and mixtures thereof, said x is from about 1 to about 30 mole percent, and said y is from about 70 to about 99 mole percent.

16. A photoconductor in accordance with claim 2 wherein said photogenerating layer is comprised of at least one photogenerating pigment and a resin binder; and wherein said photogenerating layer is situated between said substrate and said charge transport layer.

17. A photoconductor in accordance with claim 2 further including in said charge transport layer an antioxidant comprised of at least one of a hindered phenolic and a hindered amine.

32

18. A photoconductor in accordance with claim 2 further including a hole blocking layer, and an adhesive layer, wherein the hole blocking layer is in the form of a coating in contact with the supporting substrate, and the adhesive layer is in the form of a coating in contact with the hole blocking layer.

19. A photoconductor in accordance with claim 2 wherein the ratio of said second polycarbonate binder to said spirobifluorene polycarbonate to a said charge transport layer of N,N'-diphenyl-N,N'-bis(3-methylphenyl)-1,1'-biphenyl-4,4'-diamine is 54/6/40.

20. A photoconductor in accordance with claim 2 wherein said second polycarbonate is poly(4,4'-dihydroxy-diphenyl-1,1'-cyclohexane) carbonate, and said copolymer is represented by



wherein x is equal to 6 mole percent, y is equal to 94 mole percent, and said charge transport layer includes an aryl amine.

21. A photoconductor in accordance with claim 1 wherein said charge transport layer is comprised of a hole transport component, said spirobifluorene copolymer as a first resin binder, a polycarbonate second resin binder, and which photoconductor further contains a hole blocking layer in contact with said substrate and an adhesive layer in contact with said hole blocking layer.

22. A photoconductor in accordance with claim 21 wherein said polycarbonate second resin binder is a polycarbonate Z or a polycarbonate A present in an amount of from about 40 to about 60 weight percent.

23. A photoconductor in accordance with claim 1 further including a hole blocking layer, and an adhesive layer, and wherein said charge transport layer contains a charge transport component, said spirobifluorene polycarbonate binder, and a second polycarbonate dissimilar than said spirobifluorene polycarbonate, and wherein said spirobifluorene polycarbonate is represented by the following



33



-continued

34



20

wherein x and y represent mole percents, and where the sum thereof is 100 mole percent, and which spirodilactam is present in an amount of from about 3 to about 12 weight percent.

propionate, (N,N'-dimethyl 3-amino)propyl triethoxysilane, N,N-dimethylaminophenyl triethoxysilane, trimethoxysilyl propyldiethylenetriamine, and mixtures thereof, said spirodilactam polycarbonate is of the following formulas/structures



**24.** A photoconductor in accordance with claim **23** wherein the ratio of said second polycarbonate to said spirodilactam polycarbonate to said charge transport layer component is 54/6/40.

**25.** A photoconductor in accordance with claim **1** wherein said spirodilactam polycarbonate copolymer is a polycarbonate copolymer of said spirodilactam, and a bisphenol selected from the group consisting of bisphenol A and bisphenol Z.

**26.** A photoconductor comprised in sequence of a supporting substrate, a hole blocking layer thereover, an adhesive layer, a photogenerating layer, and a charge transport layer, and wherein said charge transport layer contains a charge transport component, a spirodilactam polycarbonate present in an amount of from about 1 to about 20 weight percent, and a polycarbonate present in an amount of from about 40 to about 65 weight percent.

**27.** A photoconductor in accordance with claim **26** wherein said hole blocking layer is comprised of an aminosilane of at least one of 3-aminopropyl triethoxysilane, N,N-dimethyl-3-aminopropyl triethoxysilane, N-phenylaminopropyl trimethoxysilane, triethoxysilylpropylethylene diamine, trimethoxysilylpropylethylene diamine, trimethoxysilylpropyldiethylenetriamine, N-aminoethyl-3-aminopropyl trimethoxysilane, N-2-aminoethyl-3-aminopropyl trimethoxysilane, N-2-aminoethyl-3-aminopropyl tris(ethylethoxy)silane, p-aminophenyl trimethoxysilane, N,N'-dimethyl-3-aminopropyl triethoxysilane, 3-aminopropylmethyl diethoxysilane, 3-aminopropyl trimethoxysilane, N-methylaminopropyl triethoxysilane, methyl[2-(3-trimethoxysilylpropylamino)ethylamino]-3-

wherein said x is a number of from between about 2 and about 10, and said y is a number of from between about 90 and about 98, and said polycarbonate present in an amount of from about 40 to about 65 weight percent is selected from the group consisting of poly(4,4'-dihydroxy-diphenyl-1,1-cyclohexane) carbonate, poly(4,4'-isopropylidene-diphenylene) carbonate, poly(4,4'-cyclohexylidene diphenylene) carbonate, and poly(4,4'-isopropylidene-3,3'-dimethyl-diphenyl) carbonate.

**28.** A photoconductor in accordance with claim **26** wherein said hole blocking layer is comprised of an aminosilane represented by



wherein R<sub>1</sub> is an alkylene; R<sub>2</sub> and R<sub>3</sub> are alkyl, hydrogen, or aryl, and each R<sub>4</sub>, R<sub>5</sub> and R<sub>6</sub> is alkyl.

**29.** A photoconductor in accordance with claim **26** wherein said spirodilactam polycarbonate is present in an amount of from about 3 to about 10 weight percent.

**30.** A photoconductor comprised of a photogenerating layer comprised of a photogenerating pigment, a hole blocking layer, an adhesive layer, and a charge transport layer, and wherein said charge transport layer is comprised of a charge transport component, a spirodilactam polycarbonate copolymer represented by

35



36



wherein x and y represent mole percents, and where the sum of x and y thereof is 100 mole percent, and a polycarbonate selected from the group consisting of poly(4,4'-dihydroxy-diphenyl-1-1-cyclohexane) carbonate, poly(4,4'-isopropylidene-diphenyl) carbonate, and mixtures thereof.

31. A photoconductor in accordance with claim 30 wherein said spirodilactam polycarbonate is present in an amount of from about 1 to about 20 weight percent.

32. A photoconductor in accordance with claim 30 wherein said spirodilactam polycarbonate is present in an amount of

30 from about 3 to about 15 weight percent, and said polycarbonate selected from the group consisting of poly(4,4'-dihydroxy-diphenyl-1-1-cyclohexane) carbonate, poly(4,4'-isopropylidene-diphenyl) carbonate, and mixtures thereof is present in an amount of from about 40 to about 70 weight percent.

\* \* \* \* \*